

Patented Oct. 11, 1938

2,132,463

# UNITED STATES PATENT OFFICE

2,132,463

## MANUFACTURE OF ARTIFICIAL MATERIALS

Donald Finlayson and Ronald Bezant, Spondon,  
near Derby, England, assignors to Celanese Cor-  
poration of America, a corporation of Delaware

No Drawing. Application November 3, 1936, Se-  
rial No. 108,966. In Great Britain December 14,  
1935

### 4 Claims. (Cl. 28—1)

This invention relates to improvements in the manufacture of artificial materials, and particularly improvements in the manufacture of crêpe fabrics containing crêpe threads of cellulose acetate or other organic derivative of cellulose.

Crêpe fabrics are generally produced by weaving fabrics containing weft and/or warp threads which are highly twisted, for example which have a twist of 50, 60 or more turns per inch, and subjecting the fabrics after weaving to a treatment, for example a scouring treatment, which causes the highly twisted threads to swell.

It has now been discovered that crêpe fabrics having improved properties, and particularly a much improved handle, may be obtained by subjecting the fabrics before the crêping treatment to a dry cleaning operation. Any suitable dry cleaning agent may be employed, for example a halogenated hydrocarbon such as carbon tetrachloride, trichlorethane, tetrachlorethane, trichlorethylene or perchlorethylene or a hydrocarbon such as benzene, petrol or petroleum ether. If the agent tends to swell the threads and cause crêping it is preferably diluted with a suitable liquid to a degree sufficient to prevent substantial swelling.

The process of the present invention is particularly valuable in the production of improved crêpe fabrics wherein the crêpe threads have a basis of cellulose acetate, but it is also applicable to the production of fabrics containing crêpe threads of other organic derivatives of cellulose, for example cellulose propionate, cellulose butyrate, cellulose nitroacetate, cellulose acetate-propionate and other esters and mixed esters of cellulose, methyl, ethyl and butyl celluloses and other cellulose ethers and mixed ethers and ether-esters of cellulose, for example ethyl cellulose acetate and oxy-ethyl cellulose acetate. The threads may be made of continuous or discontinuous filaments, e. g. those prepared by the processes of U. S. applications S. Nos. 726,264, filed 18th May, 1934, and 23,804, filed 28th May, 1935. The fabrics may consist solely of threads of organic derivatives of cellulose or they may also contain threads of other suitable textile materials, such for example as cotton and regenerated cellulose.

The crêpe threads employed in the production of the fabrics treated according to the present invention may be produced in any suitable manner, for example by dry twisting the threads to a suitable degree. However, threads which have been twisted in the presence of steam or hot water, e. g. as described in U. S. applications S.

Nos. 746,135, filed 29th September, 1934, and 4,085, filed 31st January, 1935, until they have, e. g. a twist of 60 to 90 or more turns per inch, have been found to give particularly valuable crêpe fabrics.

In order to improve the handle of the fabrics still further, the crêpe yarns may be lubricated before weaving with a suitable lubricating agent, for example glycerol, diethylene glycol or other polyhydric alcohol or a methyl, ethyl or other ether thereof, an oil, for example olive oil, or a suitable salt, for example triethanolamine oleate or triethanolamine abietate.

After weaving the fabrics are dry cleaned, for example with one of the agents mentioned above, and are then subjected to suitable treatment to develop a crêpe effect, for example by subjecting them to a hot aqueous treatment. Preferably the crêping operation is carried out shortly after the dry cleaning process. In this manner, as stated above, crêpe fabrics having an improved handle may be obtained. Moreover, their lustre may be improved and made to resemble that of real silk.

The following is an example of the production of a cellulose acetate crêpe fabric by the process of the present invention:

#### Example

A cellulose acetate fabric is woven which contains as weft a lubricated crêpe yarn prepared by twisting in steam to a twist of about 60-80 turns per inch.

The woven fabric is dry cleaned by treatment with perchlorethylene for 15-30 minutes and is then scoured in a dilute soap solution for about  $\frac{1}{2}$  hour at approximately 98° C. A fabric having a good crêpe figure and soft handle is thus obtained.

Having described our invention what we desire to secure by Letters Patent is:

1. Process for the production of crepe fabrics containing crepe yarns of cellulose acetate or other organic derivative of cellulose, which comprises subjecting the fabric to a dry cleaning operation without effecting a swelling of said yarns, and then subjecting the fabric to a creping operation.

2. Process for the production of crepe fabrics containing crepe yarns of cellulose acetate or other organic derivative of cellulose, which comprises subjecting the fabric to a dry cleaning operation without effecting a swelling of said yarns, said operation being carried out with a

hydrocarbon, and then subjecting the fabric to a creping operation.

3. Process for the production of crepe fabrics containing crepe yarns of cellulose acetate or other organic derivative of cellulose, said fabric containing a lubricated crepe yarn, which comprises subjecting the fabric to a dry cleaning operation which removes lubricant from said crepe yarn without effecting a swelling of said yarns, and subsequently subjecting the fabric to a creping operation.

4. Process for the production of crepe fabrics containing crepe yarns of cellulose acetate or other organic derivative of cellulose which have been twisted in the presence of a hot fluid medium, which comprises subjecting the fabric to a dry cleaning operation without effecting a swelling of said yarns, and subsequently subjecting the fabric to a creping operation.

DONALD FINLAYSON. 10  
RONALD BEZANT.